# EUROPEAN PATENT SPECIFICATION

(11) **EP 0 003 481 B1**
(45) Date of publication and mention of the grant of the patent: **27.10.1982**
(21) Application number: 78101807.2
(22) Date of filing: 21.12.1978
(51) Int. Cl.: D21H 3/78, D21D 3/00, C08J 5/18

(54) **Highly filled sheets and method of preparation thereof**
Hochgefüllte Blätter und Verfahren zu ihrer Herstellung
Feuilles fortement chargées et procédé pour leur préparation

(30) Priority: 02.02.1978 US 874458
(43) Date of publication of application: 22.08.1979
(73) Proprietor: DOW CHEMICAL (EUROPE) S.A., CH-8810 Horgen (CH)
(72) Inventor: McReynolds, Kent Bruce, Midland Michigan (US)
(74) Representative: Weickmann, Heinrich, Dipl.-Ing.

## Description

### Background of the invention

### 1. Field of the invention

The invention is concerned with pigmented, non-woven, fibrous sheets, particularly highly filled sheets having a low fiber content.

### 2. Description of the prior art

Paper has been described as a sheet material made up of many small discrete fibers (commonly cellulosic) bonded together. Small amounts of latex have been used in the paper making process. Fillers have also been used to improve certain properties of the paper even though the strength of the sheet is thereby reduced. The amount of fillers heretofore used in paper making processes on common equipment such as the Fourdrinier machine generally has not been greater than 30 or 35 percent of the total dry weight of the sheet, although up to 40 percent has been disclosed as operable. The retention of fillers in the sheet during formation has been recognized as a significant problem.

The use of asbestos in the preparation of other kinds of fibrous sheets has been practiced for many years. Such fibrous sheets have been used advantageously in the preparation of products such as floor coverings and muffler paper. However, evidence has been found that asbestos fibers are injurious to human health. In some countries, the use of asbestos has been banned and in the United States rather severe restrictions on its use are being contemplated. Accordingly, new systems which do not use asbestos are greatly desired. Such new asbestos-free systems can advance the state of the art even though on balance their properties do not exceed those of the asbestos-containing materials. Where the properties or methods'of preparation are improved, such systems would be of great benefit.

It would be especially advantageous if a new process for making highly filled papers and especially asbestos-free products could be carried out on existing equipment so that large, new capital investments would not be required.

### Summary of the invention

The process and product of this invention includes the combination of a water-dispersible fiber, a film-forming, water-insoluble, organic polymer and an inorganic filler in the form of a water-laid sheet.

According to the present invention a method for preparing a highly-filled fibrous sheet comprising the following steps:
(I) obtaining an aqueous dispersion of water dispersible fibers;
(II) mixing said dispersion therewith:
   (A) a finely-divided, substantially water-insoluble, non-fibrous, inorganic filler; and
   (B) a binder containing a fiim-forming, water insoluble, organic polymer in the form of an ionically stabilized latex;
(III) colloidally destabilizing the resulting mixture to form a fibrous agglomerate in aqueous suspension;
(IV) distributing and draining said aqueous suspension on a porous support to form a wet web;. and
(V) drying the web; is characterized by the fact that the mixture obtained in step (II) contains:
   from 1 % to 3096 of fibers,
   from 60% to 95% of fitter.
   from 2% to 30% of latex, said percentages being on dry weight basis, calculated on the total dry weight, and that the ionically stabilized latex is devoid of sufficient non-ionic stabilization to interfere with the formation of a fibrous agglomerate.

Significant features of the process and product are a low proportion of fiber and a high proportion of inorganic filler as well as good runnability of the process on common paper-making equipment and the good properties of the product. The preferred highly filled, water-taid, fibrous, asbestos-free sheets are suitable as a replacement or substitute for asbestos sheets in many of their applications but are not restricted to such uses. Representative uses of the sheets are as muffler paper, underlayment felt for vinyl floor covering, gasket papers, roofing paper, sound-deadening paper, pipe wrap, insulation paper, heat deflection papers, cooling tower packing, electrically resistant paper and board products.

### Description of the preferred embodiments

The product and process of this invention requires a water-dispersible fiber, a film-forming, water-insoluble, organic polymer and a finely-divided, substantially water-insoluble, non-fibrous, inorganic filler. In the preferred process, a flocculating agent also is required.

The fiber is any water-insoluble, natural or synthetic water-dispersible fiber or blend of such fibers. Usually water-dispersibility is provided by a small amount of ionic or hydrophilic groups or charges which are of insufficient magnitude to provide water-solubility. Either long or short fibers, or mixtures thereof, are useful, but short fibers are preferred. Many of the fibers from natural materials are anionic, e.g., wood pulp. Some of the synthetic fibers are treated to make them slightly ionic, i.e., anionic or cationic. Glass fibers, chopped glass, blown glass, reclaimed waste papers, cellulose from cotton and linen rags, mineral wool, synthetic wood pulp such as is made from polyethylene, straws, ceramic fiber, nylon fiber, polyester fiber, and similar materials are useful. Particularly useful fibers are the cellulosic and lignocellulosic fibers commonly known as wood pulp of the various kinds from hardwood and softwood such as stone ground wood, steam-heated mechanical pulp. chemimechanical pulp, semichemical pulp and chemical pulp. Specific examples are unbleached sulfite pulp, bleached sulfite pulp, unbleached sulfate pulp and bleached sulfate pulp.

The film-forming, water-insoluble, organic polymer use_{T}ul in the practice of this invention is natural or synthetic and may be homopolymer, a copolymer of two or more ethylenically unsaturated monomers or a mixture of such polymers. Particularly for ease of processing to make the product and for limiting the loss of pollutants to the surroundings, it is generally advantageous that the polymer is in the form of a latex, i.e., an aqueous colloidal dispersion. Representative organic polymers are natural rubber, the synthetic rubbers such as styrene/butadiene rubbers, isoprene rubbers, butyl rubbers and nitrile rubbers and other rubbery or resinous polymers of ethylenically unsaturated monomers which are film-forming, preferably at room temperature or below, although in a particular instance a polymer may be used which is film-forming at the temperature used in preparing that sheet. Non-film-forming polymers may be used in blends provided that the resulting blend is film-forming. Polymers which are made film-forming by the use of plasticizers also may be used. Polymers which are readily available in latex form are preferred-especially hydrophobic polymers which are prepared by emulsion polymerization of one or more ethylenically unsaturated monomers. Representative of such latexes are those described in US-A-3,640,922, from column 1, line 61, to column 2, line 34. That passage (particularly column 2, lines 2-9) indicates a preference for latexes of polymers and copolymers not having a substantial proportion of hydrophilic groups. For use in the present invention, the latexes preferably have some ionic hydrophilic groups but must be devoid of sufficient non-ionic colloidal stabilization which would interfere with formation of the fibrous agglomerate. Such non-ionic, colloidal stabilization could be provided by non-ionic emulsifiers or by the presence of copolymerized monomers having the kinds of hydrophilic groups as are found in non-ionic emulsifiers, for example, hydroxyl and amide groups. Thus, if monomers having such hydrophilic groups are polymerized constituents of the latex polymers, such monomers will be present in small proportions such as less than about 10 percent, usually less than about 5 percent of the polymer weight for best results. Also, while very small amounts of non-ionic emulsifiers can be tolerated in some compositions, their use ordinarily is not advantageous and they should not be used in amounts sufficient to interfere with the destabilization step of the process.

Latex compositions for use in this invention are selected from latexes in which a polymer of the foregoing description is maintained in aqueous dispersion by ionic stabilization. Such ionic stabilization is obtained, for example, by use of an ionic surfactant or small amounts of a monomer containing an ionic group during emulsion polymerization to prepare the latex. The small amount of ionic groups which are bound to the polymer generally will provide less than about 0.7 milliequivalent of charge per gram of polymer in the latex. Ordinarily it is preferred that the latex component for this invention have a charge bound to the polymer of from about 0.03 to about 0.4 especially from about 0.09 to about 0.18, milliequivalent per gram of polymer in the latex, particularly when the charge is provided by carboxylic salt groups. The term "bound to the polymer" with respect to ionic groups or charges refers to ionic groups or charges which are not desorbabie from the polymer. Materials containing such ionic groups or charges may be obtained as noted above by copolymerization of a monomer containing ionic groups or by other ways such as grafting, by attachment (through covalent bonds) of catalyst fragments to the polymer, especially sulfate groups from persulfate catalysts, or by the conversion to ionic groups of non-ionic groups already attached to the polymer by covalent bonds.

The ionic groups advantageously are the carboxyl salt groups, especially the alkali metal and ammonium carboxylate groups, or quaternary ammonium salt groups, but other anionic and cationic groups are useful; for example, sulfate, sulfonate and amino groups. Carboxyl salt groups are especially advantageous.

For latex compositions having little or no detectable amount of ionic groups bound to the polymer, the ionic stabilization is provided by adsorbed ionic surfactants; Small amounts of ionic surfactant can be used with latexes having bound ionic groups but increasing amounts of surfactants above the amounts required for adequate stabilization tend to make proper selection of other components of the system more critical and complicate the formulation,

Anionic and cationic surfactants are well known in the art and suitable materials of those classes can be selected, for example, from among those listed in the annual issues of "McCutcheon's Detergents and Emulsifiers" such as the 1973 issue, published by McCutcheon's Division, Allured Publishing Corporation, Ridgewood, NJ. Examples of non-ionic surfactants are also provided in the above-noted reference.

The especially preferred latexes (i.e., latexes having from about 0.09 to about 0.18 milliequivalent of bound charge per gram of polymer) generally work best in the process and provide overall the best composite sheet. When these especially preferred latexes are used in the process, the procedure for the colloidal destabilizing step as well as the selection of the amount and kinds of the other ingredients within the limits described herein are less demanding. With such latexes, observation of the behavior during the process provides guidance for selections of the various other components for use when it is desired to use latexes within the preferred and operable limits but outside the especially preferred limits. For illustration, in carrying out the colloidal destabilizing step by the method using a flocculant opposite in charge to the latex, the appearance and nature of the resulting flocculated material when using the especially preferred latexes will guide the skilled in the art in the critical sqlection of the other components when a latex outside the especially preferred but within the operable limits is used- especially with the higher bound charge latex.

There are instances where for particular purposes, however, it is preferred to use the latexes having a bound charge above 0.18 and even above 0.4 milliequivalent of charge per gram polymer in the tatex, e.g., where the bound charge is cationic, where rebrokability of the composition is desired, or where the bound ionic groups in addition to their stabilization role are desired in larger amounts to perform other advantageous interactions with other components of the composition.

The charge/mass ratio, expressed herein as milliequivalents of charge per gram of polymer in the tatex, does not necessarily (and generally does not) correspond, for example, to the proportion of milliequivalents of monomer containing an ionic group which is copolymerized with the non-ionic, hydrophobic monomers by emulsion polymerization to form the latex. These differences arise (1) because some of the ionic monomer is polymerized inside a latex particle and thus is not effective in stabilizing the dispersion of polymer particles and is not measured, (2) the ionic monomer may homopolymerize or copolymerize to form varying amounts of water-soluble polymers, or (3) in some instances the ionic monomer does not polymerize as completely as the other monomers. In general, as the proportion of the ionic monomer in relation to the total monomer increases, the proportion of the ionic groups of the ionic monomers which are on the surface of the particle decreases and the amount buried within the latex particles or which forms ionic water-soluble polymers increases. Since too large an excess of water-soluble polymers, either anionic or non-ionic, can cause problems in the present process, it is generally desirable where bound charges at the higher levels are employed (a) to use latexes for which special precautions are taken in their preparation to minimize water-soluble polymer formation or (b) to add materials to the formulation which will insolubilize the water-soluble polymers or (c) to remove some or all of such water-soluble polymers.

Latexes of any conveniently obtainable particle size are useful in the practice of this invention but average particle diameters of from about 1000 to about 2600 angstroms are preferred-especially from about 1200 to about 1800 angstroms. Since the latex is diluted during the process, the solids content of a latex as supplied is not critical.

In the preparation of many of the latexes of different compositions useful in the invention, it is advantageous to use a chain transfer agent of known kinds such as, but not restricted to, the various long chain mercaptans, bromoform, and carbon tetrachloride.

The fillers which are used in the practice of this invention are finely-divided, essentially water-insoluble, inorganic materials. Such materials include, for example, titanium dioxide, amorphous silica, zinc oxide, barium sulfate, calcium carbonate, calcium sulfate, aluminum silicate, clay, magnesium silicate, diatomaceous earth. aluminum trihydrate, magnesium carbonate, partially calcined dolomitic limestone, magnesium hydroxide and mixtures of two or more of such materials. Magnesium hydroxide runs particularly well on common, available paper-making equipment to form a product having good properties, contributes to flame resistance and to resistance to microbiological attack and is preferred. However, calcium carbonate is sometimes preferred, especially in uses where the economic factors are particularly important, because it is readily available, provides good structure, runs well in the process and the impure grades, such as ground limestone, can be used. The particle size of the fillers is such that the preponderant proportion is below 50 microns in diameter. The average diameter is generally above about 0.1 micron aid preferably is from about 0.1 to about 20 microns. For preferred embodiments the fillers should be free of asbestos contaminants.

In many embodiments of the process of this invention, a flocculating agent or destabilizing agent (sometimes also called a deposition aid) is highly advantageous. Such flocculating agents are water-dispersible, preferably water-soiuble, ionic compounds or poiymers, i.e., compounds or polymers having a positive or a negative charge. For the process, ordinarily a flocculating agent is chosen which has a charge opposite in sign to the ionic stabilization of the latex. If the latex has a negative charge, the flocculating agent will have a cationic charge and vice versa. However, when combinations of two or more flocculating agents are used, not all of them are necessarily opposite in charge to the initial charge of the latex.

Representative flocculants are cationic starch; water-soluble, inorganic salts such as alum, aluminum sulfate, calcium chloride and magnesium chloride; an ionic latex having a charge opposite in sign (+ or -) to that of the winder latex, e.g., a cationic latex or an anionic latex; water-soluble, ionic, synthetic, organic polymers such as polyethyleneimine and various ionic polyacrylamides such as carboxyl-containing polyacryamides; copolymers of acrylamide with dimethyfaminoethyl methacrylate or diallyldimethyl ammonium chloride; polyacrylamides modified other than by copolymerization to have ionic groups: and combinations of two or more of the above, added simultaneously or in sequence. Quaternized poiyacrylamide derivatives are especially advantageous when the latex which is used is anionic. Polymeric flocculants are preferred because they are more efficient, tend to produce less water-sensitive products and provide better shear stability of the furnish.

The preferred process for making the products of this invention is particularly adaptable to be carried out on handsheet-forming apparatus or common, continuous paper-making equipment such as a Fourdrinier machine, a cylinder machine, suction machines such as a Rotaformer, or on millboard equipment. Suitable also for use in the practice of this invention are other well-known modifications of such equipment, for example, a Fourdrinier machine with secondary headboxes or multicylinder machines in which, if desired, different furnishes can be used in the different cylinders to vary the composition and the properties of one or more of the several plies which can comprise a finished board. For further details, reference is made to the general summary of paper and paper making as found in Kirk-Othmer, Encyclopedia of Chemical Technology, Interscience Publishers, Inc., NY 14 (1967) pages 494-510, with the sheet forming aspect and appropriate equipment therefor being described on pages 505-508.

The preferred process requires the following steps:
(1) providing an aqueous dispersion of from about 5 percent to about 15 percent, of a water-dispersible, but water-insoluble fiber;
(II) mixing therewith (A) from about 70 percent to about 90 percent, of a finely-divided, substantially water-insoluble, non-fibrous, inorganic fiter and (8) from about 5 percent to about 15 percent, of a binder containing a film-forming; water-insoluble, organic polymer in the form of an ionically stabilized latex;
(III) colloidally destabilizing the resulting mixture to form a fibrous agglomerate in aqueous suspension;
(IV) distributing and draining the aqueous suspension on a porous substrate such as a wire to form a wet web; and
(V) drying the web.

The foregoing percentages are on a weight basis calculated on the total dry weight.

In the practice of this invention, the fibrous material is subjected to mechanical action in the presence of water in a manner variously described in the paper-making art as pulping, beating, or refining. Cellulosic fibers for this invention ordinarily are refined to a Canadian Standard Freeness (CSF) at 0.3 percent consistency of from about 300 milliliters to about 700 milliliters, preferably from about 400 milliliters to about 600 milliliters. Synthetic fibers are similarly mechanically treated but unless specially treated do not fibrillate to give the same degree of dispersion as is obtained with cellulosic pulps so that the Canadian Standard Freeness test is not particularly adapted to such materials. The synthetic fibers generally have a fiber length up to about 9,5 mm preferably from about 3,17 mm to about 6,35 mm.

· The consistency (percentage by weight of dry fibrous material) of the stock thus obtained ordinarily is from about 0.1 percent to about 6 percent, preferably from about 0.5 percent to about 3 percent.

In the mixing of the fiber with other components of the sheet, additional water is included to reduce the consistency of the resulting furnish to a value ordinarily within the range of from about 0.1 percent to about 6 percent, preferably from about 1 percent to about 5 percent. Part of the water of dilution advantageously is white water, or process water, recycled from later steps in the sheet-making process. Alternatively or additionally, some of the process water can be used in the step of refining the fiber. Ordinarily the filler, the dilution water and the latex. generally prediluted to a lower solids content than at which it was manufactured, are added (usually but not necessarily in that order) to the fiber dispersion with agitation. At least some of the required colloidal destabilization can occur simultaneously with the mixing of the fiber, filler and latex either through interaction of the required components or through the concurrent addition of other optional wet-end additives such as those mentioned below. The mechanical shear caused by mixing and by transfer of the materials through the equipment used can cause, or assist in, the destabilization. However, the combination of the mixing and the destabilization steps produce a fibrous agglomerate in aqueous suspension, which at a concentration of 100 grams of solids in 13,500 milliliters of the aqueous suspension, should drain in a time of from about 4 seconds to about 120 seconds, especially from about 1 5 seconds to about 60 seconds and preferably from about 30 seconds to about 45 seconds in a 25,4 cm by 30,5 cm Williams Standard Sheet Mould, having a 5,08 cm outlet and a 76,2 cm water leg and fitted with a standard 100-mesh, stainless steel screen (wire size, 0,114 mm) to provide in one pass at least 85 percent retention of solids which contain at least 60 percent by weight of filler. Additionally, in the preferred embodiments, the drainage water is substantially clear. An effective and preferred method of carrying out (or completing the.carrying out) of the destabilization is the mixing with the. other components a flocculating agent, i.e., a water-dispersibie or water-soluble, ionic compound having a charge opposite in sign (+ or -) to that of the ionic stabilization in a sufficient amount, such an amount generally being less than about 1 percent, based on the total dry weight of the components. When used, a flocculant is added so that the destabilization can take place before the distributing and draining step. With continuous sheet-making apparatus such as the Fourdrinier paper machine, the flocculant is added at the stock chest or at such a point in the stock transfer portion of the apparatus that there is sufficient time for the desired action to take place yet not so much that the resulting flocculated stock is subjected to undue shear. After distributing and draining the resulting aqueous dispersion, the wet web obtained thereby optionally is wet-pressed and then dried with equipment conventionally used in paper-making.

The temperature of the process through the step of forming the wet web usually is in the range of from about 4.4°C to about 54°C although temperatures outside those ranges can be used provided that they are above the freezing point of the aqueous dispersion and are below the temperature at which the latex polymer being used would soften unduly. Sometimes temperatures above ambient conditions promote faster drainage.

Also useful in the practice of this invention are small amounts of various other wet end additives of the types commonly used in paper-making. Such materials include antioxidants, various hydrocarbon and natural waxes, particularly in the form of anionic or cationic emulsions; cellulose derivatives such as carboxymethyl cellulose and hydroxyethyl cellulose; water-soluble organic dyestuffs, water-insoluble but water-dispersible coloring pigments such as carbon black, vat colors and sulfur colors; starch, natural gums such as guar gum and locust bean gum, particularly their anionic and cationic derivatives: non-ionic acrylamide polymers; strength improving resins such as melamine-formaldehyde resins, ureaformaldehyde resins and curing agents of various types such as the sulfur-containing vulcanizing agents and accessory compounds. Further quantities and/or kinds of anionic or cationic surfactants may also be added in small amounts at various points in the process if desired. Non-ionic surfactants should be used sparingly, if at all.

Optionally, either internal or external sizing can be employed together with the required features of this invention.

The densities of the products obtained from the above-described process cover a wide range, such as from about 0,48 g/cm³ to about 2,4 g,lcm3..

Since the filler constitutes such a high proportion of the weight of the products, the identity of the filler ejected for a particular product has considerable effect on the density and other properties of the product.

The thickness of the sheet which is produced can vary from about 0,076 mm to about 3,17 mm, the preferred value depending somewhat upon the proposed use. However, the thickness generally is from about 0,38 mm to about 1,65 mm.

The method of this invention results in production of water-laid, self-supporting sheets at high filler loading with a high proportion of the filler which is added being retained in the sheets. As commonly used in the art, the term "water-laid sheet" refers to a sheet which is deposited from a dilute aqueous suspension, usually having a solids content of four percent or less. While the filler constitutes the major proportion of the sheet, the latex and fiber are also retained in the sheet in high proportions. Retention in the sheet of all of the solids used in the process generally is greater than 85 percent by weight and in the preferred embodiments is greater than 95 percent

The process and product of this invention has many advantages. In comparison with paper sheets of the prior art, there is less moisture in the sheet when it comes off the wet end of the machine. Hence, with the same bases weight of the sheet, less energy is required to dry the sheet and the machine can be run faster or a thicker sheet can be dried. The new process can be carried out using presently designed and available equipment of the kind commonly owned by paper manufacturers. Readily available raw materials are used. A large proportion of the raw materials is inexpensive filler and the total cost is low. The density can be altered simply by the choice of filler. The preferred embodiments also are asbestos-free.

The following examples illustrate ways in which the present invention may be carried out, but should not be construed as limiting the invention. All parts and percentages are by weight unless otherwise expressly indicated. Components identified by letter designations, e.g., Latex A, are described in Tables A, B, C and D.

In the examples where handsheets are made, a specially-developed standard procedure is used with such modifications as are shown in specific examples. In. the standard procedure, the indicated fiber (if cellulosic) is pulped to a Canadian Standard Freeness (CSF) of 500 milliliters and a consistency of about 1.2 percent by weight. The synthetic fibers are dispersed in water with a TAPPI disintegrator (600 counts) but a Canadian Standard Freeness measurement is not made. With a sufficient quantity of the resulting aqueous dispersion to provide 5 grams of the fiber, dry basis, is mixed an additional precalculated amount of water to give a final volume of 2000 milliliters. Stirring is continued while 80 grams of the indicated filler is added as a powder except where shown as an aqueous slurry, followed by 15 grams, solids basis, of the indicated latex. The resulting mixture is mechanically sheared for 15 seconds in a Jabsco centrifugal pump followed by agitation with a laboratory stirrer having two 3- bladed propellers on one shaft operated at 900 rpm while a 0.1 percent solution or her indicated flocculant is added slowly until the water phase is essentially clear. A sufficient amount about 62 ml) of .the resulting furnish to provide 3 grams of solids is diluted to 1000 milliliters with water and the Canadian Standard Freeness is.measured according to TAPPI Standard T 227-M-58. The freeness. sample is returned to the furnish which is then diluted to 13,500 milliliters and a sheet is formed in a 25,4 cm by 30,5 cm Williams Standard Sheet Mould and the drainage time on a 100-mesh screen is recorded. The resulting wet sheet is couched from the wire in a press at approximately 0,7 kg/cm² using two blotters to absorb water from the sheet. The sheets are stacked alternately with blotters and wet pressed at 35,2 kg/cm².

The partially dried sheets are then weighed and dried on a sheet dryer at a platen temperature of 116⁰ to 121 °C, alternating sides of the sheet against the platen at 0.5 to 1-minute intervals. The resulting dried sheets are weighed to determine the total solids which are retained in the sheet. Since sufficient materials are used to make a 100-gram sheet on complete retention, the dry weight also represents the percent retention.

### Examples 1-14

Handsheets are prepared from the designated latex, unbleached southern pine kraft and the designated fillers using Flocculant A by the standard procedure described above except as indicated. The data for the preparation of the sheets are shown in Table 1. The properties of the sheets are shown in Table II.

### Examples 15-42

Handsheets are prepared from the designated latex, the designated kind of fiber pulped to the designated Canadian Standard Freeness (CSF), the designated filler and the designated flocculant by the standard procedure described above except as indicated. Sheet preparation data are shown in Table III and the sheet properties in Table IV.

### Examples 43-46

Handsheets are prepared by the standard procedure described above wherein the fiber is Fiber D, and the filler, latex and flocculant are the kinds specified in Table V. Sheet properties are shown in Table VI.

### Examples 47-49

Handsheets are prepared by the standard procedure described above wherein the fiber is unbleached softwood kraft, the latex is Latex B, the filler is Filler A, and the flocculant is as specified. In addition of the flocculant. the indicated amount of alum was added first and stirred for one minute, then a sufficient amount of the other flocculant to complete flocculation was added. Data for preparation of the handsheets are shown in Table Vil. Properties of the sheets are shown in Table VIII.

### Examples 50-53

Handsheets are prepared by the standard procedure described above wherein the fiber, latex, and flocculant are as shown and the filler is Filler A in the amount as shown. Data for the sheet preparation are shown in Table IX. Samples of the sheets are placed in a tropical chamber maintained at 100 percent relative humidity and 32.2°C which has previously been inoculated with organisms including Aspergillus niger, Trichoderma viridie, Aureobasidium pullulans, Chaetomium globosum and unidentified species of Penicillium. At the end of 21 days and 49 days, the samples are checked for visible evidence of microbiological attack and room temperature tensile loss values are measured on strips 7,6 cm long over a 2,54 cm span of the samples. For comparison, handsheets are prepared from 85 parts of asbestos (Johns Manville, Paperbestos No. 5) and 15 parts of Latex C (Comparative Example A-1) and 85 parts of asbestos and 15 parts of Latex B (Comparative Example A-2). Test data are shown in Table X.

The visual rating is based on an arbitrary scale for visible evidence of microbiological attack as follows:
O=no attack
1=very slight attack
2=slight attack
3=moderate attack
4=heavy attack
5=very heavy attack

The tensile tests are carried out, with the exception of the length of the test strip, in the manner described after all the examples. The tensile data recorded in Table X is the percent change in tensile between the test strips and control strips of the same kind which are prepared at the same time and are held for the same period outside the tropical chamber.

### Examples 54-60

Handsheets are prepared by the standard procedure described above except that different ratios of fiber, latex and filler are used. The fiber is unbleached softwood k,aft, the latex is Latex B, the filler is Filler B and the flocculant is Flocculant A. Data are shown in Table XI.

### Examples 61-82

A handsheet (Example 61) is prepared from unbleached softwood kraft, Latex F, Filler 0 and flocculant A by the standard procedure described above. Another handsheet (Example 62) is prepared in the same manner except that 0.25 part of a cationic polyamideepichlorohydrin resin (Kymene 557) is added as a 0.132 percent aqueous solution to the aqueous fiber dispersion before mixing with the filler and latex. Data are shown in Table XII.

### Examples 63-64

Handsheets are prepared from Latex N, Fiber R, and the designated filler using Flocculant E in the amount according to the standard procedure except that a wet-strength additive, which is a polyamide-epichlorohydrin resin having ₁₂.₈ percent nitrogen, is added after the filler in the shown in Table XIII, and 1 percent total solids basis, of an anionic emulsified hydrocarbon wax the latex. A summary of data is provided in Table XIII.

The products from these examples in view of their properties, especially dimensional stability in the presence of water, are particularly adapted for use in flooring compositions.

### Examples 65-70

Using the standard procedure except that the step of mechanically shearing on a Jabsco centrifugal pump was omitted, handsheets are prepared from the designated latex, Fiber E and Filler Q using Flocculant E in the proportions shown in Table XIV for the latex, fiber and flocculant and the amount of filler is the difference between 100 percent and the total of latex and fiber, all on a dry solids basis. Also the amounts are chosen such as to provide handsheets theoretically weighing 75 grams rather than 100 grams and the dilution water of the furnish is reduced correspondingly. Data are shown in Table XIV.

### Example 71 and comparative example 71-C

With a portion of Latex R is blended 8 percent (based on the solids content of the latex) of carbon tetrachloride. The resulting product is centrifuged. The aqueous serum is removed and the remaining solids are washed with water. The resulting damp solids are redispersed in water by subjecting the solids and water to vigorous agitation for from 30 minutes to one hour. The resulting dispersion is Latex R-1 and has a pH of 3.8.

Except for using quantities theoretically sufficient to prepare a 30-gram sheet rather than a 100- gram sheet and correspondingly reducing the dilution water of the furnish, the standard process for preparing handsheets is used with each of Latex R and Latex R-1 in a proportion of 15 percent of the respective latex, 15 percent of Fiber E and 75 percent of Filler K (solids basis, calculated on the weight of latex, fiber and filler) using 127 milliliters of a 0.1 percent aqueous solution of Flocculant E. Damp handsheets are formed with each of Latex R-1 (Example 71) and Latex R (Comparative Example 71-C) with a drainage time of 20 seconds and 29 seconds, respectively. In Example 71 there is only a barely detectable amount of scum in preparation of the furnish with only slight sticking of the sheet to the wire when the damp handsheet is dried. During the addition of the flocculant, the progression of flocculation is easily observed. However, in comparative Example 71 ?C, a large amount of scum and froth appears in the preparation of the furnish. Such severe sticking of the dried handsheet to the wire and blotter occurs that a sheet cannot be separated from the wire.

The bound charge on Latex R and Latex R-1 is the same because the procedure to prepare Latex R-1 from Latex R would not alter the existing bound charge (from carboxyl groups). The significant difference is the removal from Latex R of water soluble components, e.g., surfactants and acrylic acid polymers or copolymers of sufficiently low molecular weight and high enough carboxyl content to be water soluble. These results are consistent with the view that too large amounts of water-soluble polymers, including surfactants and ionic polymers are deleterious in carrying out the present process.

### Examples 72 and 73

An aqueous dispersion of fiber is prepared at about 4 percent consistency from bleached southern pine kraft and water in a Black Clawson Hydrapulper. The crude dispersion is pumped to a refiner chest and refined to a Canadian Standard Freeness of 500 milliliters by recirculation through a Sprout-Waidron Twin-Flow Refiner. Highly filled sheets for Examples 72 and 73 are prepared from portions of the fiber dispersion, a latex and a filler as identified and in the proportions shown in Table XV by use of a 33-inch Fourdrinier paper machine having a phosphor bronze, long crimp wire, four flat suction boxes between the breast roll and a suction couch roll, a first wet press, a reverse press, a multi-section dryer with a size press between sections and a 7-roll calendar stack. The fiber dispersion, filler, water, and the latex diluted to 25 percent solids are added to a machine chest, in that order, with the amount of added water being calculated to provide 4 percent consistency. The resulting stock is transferred with the aid of a stock pump through a stock valve and then through a fan pump to the headbox.

The flocculant shown in Table XV is added between the stock pump and the stock valve and some white water from the later stages of the process is returned to the system between the stock valve and the fan pump so that the consistency of the furnish in the headbox is as shown in Table XV. The furnish from the headbox is fed onto the wire moving at 6.1 meter per minute where white water drains to form a wet sheet from which additional water is removed by means of the four suction boxes before the sheet is removed from the wire at the suction couch roll. After the two press stages have reduced the water-content still further, the sheet is fed through the dryer and calendar stack. Data for the process and property data for the highly filled sheets thus formed are shown in Table XV.

### Example 74

An aqueous dispersion of fiber is prepared at about 4 percent consistency from unbleached northern softwood kraft and water in a Black Clawson Hydrapulper.

The crude dispersion is pumped to a refiner chest and refined to a Canadian Standard Freeness of 500 milliliters by recirculation through a Sprout-Waldron Twin-Flow Refiner. Highly filled sheets for Example 74 are prepared from the fiber dispersion, a latex, a filler as identified and a wet strength additive which is a cationic polyamide-epichlorohydrin resin having. 12.8 percent nitrogen and a viscosity at 25°C between 0.040 and 0,065 Pa · S, all in the proportions shown in Table XVI by use of a Fourdrinier Paper Machine having (a) a 91.4 cm wide plastic wire, (b) a headbox equipped with a manifold type inlet, a homogenizer roll and a Neilson slice, (c) a suction couch roll, (d) a straight-through plain press, (e) a plain reversing press, (f) a dryer section consisting of 7 and 5 driers with integrally cast journals and 2 felt driers on the bottom and top first section felts and (g) a calendar stack consisting of 8 rolls with the intermediate rolls bored for steam. The fiber dispersion, filler, wet strength additive, water and the latex diluted to 25 percent solids are added to a machine chest, in that order, with the amount of added water being calculated to provide 4 percent consistency. The resulting stock is transferred with the aid of a stock pump through a stock valve and then through a fan pump to the headbox. The flocculant shown in Table XVI is added between the stock pump and the stock valve and some white water from the later stages of the process is returned to the system between the stock valve and the fan pump so that the consistency of the furnish in the headbox is as shown in Table XVI. The furnish from the headbox is fed onto the wire moving at 12.2 m per minute where white water drains to form a wet sheet from which additional water is removed by means of suction boxes before the sheet is removed from the wire at the suction couch roll. After the two press stages have reduced the water content still further, the sheet is fed through the dryer and calendar stack. Data for the process and property data for the highly filled sheets thus formed are shown in Table XVI.

The various tests are carried out as described below with such further modifications as are shown in specific examples.

### Canadian Standard Freeness (CSF)

The value, in milliliters, is determined according to TAPPI Standard T 227-M-58 on a sample containing 3 grams of solids diluted with water to 1000 milliliters.

### Elmendorf Tear

The test is carried out according-to TAPPI method T414-ts-65. Results are shown as an average of at least 3 samples.

### Elongation, percent

The elongation at room temperature, elongation at 177°C (hot), elongation DOP and elongation water are determined over a 15,24 cm span at the same time as the respective Tensile tests―see description below.

### Limiting Oxygen Index (L.O.I.)

The LO.!. is determined according to test method ASTM D 2863-74.

### Mullen Burst

The TAPPI test method D 403-os-76 is followed except the test is applied to thicker sheets. The results shown are an average of 4 or 5 samples.

### Retention, percent

The materials for the handsheets are added in amounts sufficient to provide sheets weighing 100 grams. Thus, the dry weight of the product also represents the percent retention of solids in the sheet

For the sheets made on the Fourdrinier machine, the percent retention relates to the proportion of filler retained in the sheet. Combustion of test samples is carried out under conditions such as to retain the residue of the filler (calculated as percent ash) but to remove the other components. The percent. ash is multiplied by an appropriate factor for changes in the filler caused by combustion (e.g., Mg(OH)2-MgO) to determine the percent filler in the sheet. From the percent filler found in the sheet and the percent filler added (solids basis), the percent retained in the sheet is calculated as an average of three samples.

### Stiffness, Taber

Taber Stiffness (g-cm) is determined according to TAPPI standard method T 489-os-76 except that test results from three samples are averaged unless otherwise stated. The value obtained is corrected to a value for 0,76 mm thickness by multiplying by the factor:

To distinguish from modified Taber stiffness tests (DOP and water―as described below), the TAPPI method is sometimes referred to herein as "Taber Stiffness, Reg.".

### Stiffness, DOP

The DOP stiffness (g-cm) is determined in the same manner as the Taber Stiffness except that the sample is soaked in dioctyl phthalate for 18-24 hours before testing and the reported value is the average of 2 samples.

### Stiffness, Water

The water stiffness is determined in the same manner as the Taber Stiffness except that the sample is soaked in water for 18-24 hours before testing and the reported value is the average of two samples.

### Tensile, room temperature (R.T.)

Sheets are cut into 2,54 cm by 20,3 cm strips and the minimum thickness over the test area is determined. The strip being tested is placed in an Instron (Trade Mark) test machine having a 15 cm span. While the Instron is operated at a head speed of one inch per minute, the elongation and pounds at break are recorded.

The kg/cm² at break are calculated by dividing the tensile at break by the thickness of the sample. Results are reported as an average of 3 samples.

### Tensile, Hot

The hot tensile is tested in the same manner as room temperature tensile except that just before the test, the test specimen is heated at a temperature of 177°C for one minute while clamped in the jaws of the test machine.

### Tensile, DOP

The DOP tensile is tested in the same manner as the room temperature tensile except that the test sample is soaked in dioctyl phthalate for 24 hours before testing.

### Tensile, Water

The water tensile is determined in the same manner as the DOP tensile, except the soaking is in water.

### Toluene pickup

A suitable specimen (5,08 cm by 10,16 cm) is soaked for 15- seconds in toluene, the weight pickup is recorded and the pickup in percent by weight is calculated.

### Kerosene Pickup

The kerosene pickup is measured in the same manner as the toluene pickup except the soaking is in kerosene.

### Water pickup

The water pickup is determined in the same manner as the toluene pickup except that the soaking is in water for 24 hours.

### Water swell

The water swell is determined in the same kind of specimen as used for the water pickup and is calculated on the increase in length of the specimen resulting from soaking in water for 24 hours.

### Charge/mass ratio

The bound charge per gram of polymer in a latex is measured by conductometric titration after the water-soluble ionic materials have been removed. If sufficient bound charge is present, the latex can be centrifuged, often after adding, for example, 3 percent (based on the latex solids) of carbon tetrachloride, the serum phase is separated, the remaining solids are washed and then redispersed by vigorous agitation in water. The conductometric titrations are made on the redispersed solids. Ion exchange methods also may be used to remove the ionic water-soluble materials from latexes having sufficient bound charge to remain stable until the conductometric titration is completed. For latexes having insufficient bound charge to remain stable, small amounts of non-ionic surtactans are added before the ion exchange procedure.

## Claims

1. A method for preparing a highly-filled fibrous sheet comprising the following steps:
(1) obtaining an aqueous dispersion of water dispersible fibers;
(II) mixing said dispersion therewith:
(A) a finely-divided, substantially water-insoluble, non-fibrous, inorganic filler; and
(B) a binder containing a film-forming, water insoluble, organic polymer in the form of an ionically stabilized latex;
(III) colloidally destabilizing the resulting mixture to form a fibrous agglomerate in aqueous suspension;
(IV) distributing and draining said aqueous suspension on a porous support to form a wet web; and
(V) drying the web;
characterized by the fact that the mixture obtained in step (II) contains:
from 1 % to 30% of fibers,
from 60% to 95% of filler,
from 2% to 30% of latex,
said percentages being on dry weight basis, calculated on the total dry weight, and that the ionically stabilized latex is devoid of sufficient non-ionic stabilization to interfere with the formation of a fibrous agglomerate..

2. The method of Claim 1 characterized by the fact that the colloidally destabilizing step forms a flbrous agglomerate in aqueous suspension having the characteristics that, at a concentration of 100 grams of solids in 13,500 milliliters, the suspension will drain in a time of from about 4 seconds to about 120 seconds in a 10-inch (25.4 cm) by 12-inch (30.5 cm) Williams Standard Sheet Mould having a 2-inch (5.1 cm) outlet and a 30-inch (76.2 cm) water leg and fitted with a 100-mesh, stainless steel screen having a wire diameter of 0,0045 inch (0.0114 cm) so that, by the draining of step (IV), one retains in the wet web at least 85% of the total solids from the fibrous agglomerate including at least 60% by weight of the filler.

3. The method of Claim 1 characterized by the fact that the organic polymer in the latex has less than 0.7 milliequivalent of bound charge per gram of polymer.

4. The method of Claim 3 characterized by the fact that the organic polymer in the latex has a bound charge of from 0.3 to 0.4 milliequivalent per gram of polymer.

5. The method of Claim 2 characterized by the facts that the aqueous dispersion of fibers has a consistency of from 0.1 % to 6%, the fibres are cellulosic fibers, and the fibrous agglomerate has a drain time of 15 to 60 seconds.

6. The method of Claim 1 characterized by the fact that amount of the fibers is from 5% to 15%, the amount of filler is from 70% to 90%, and the latex contains copolymerized styrene and butadiene.

7. The method of Claim 1 characterized by the fact that the latex is a blend of at least two different latex compositions and at least one of the latexes contains a copolymer of an ethylenically unsaturated carboxylic acid.

8. The method of Claim 1 in which the destabilizing step is carried out by mixing with the product of steps (I) and (II) a sufficient amount of a water-soluble or water-dispersible, ionic compound or poiymer having a charge opposite in sign to that of the ionic stabilization of the latex.

9. A water-laid, self-supporting sheet consisting essentially of a composite of (A) water-dispersible fibers, (B) a film-forming, water-insoluble, organic polymer, and (C) water-insoluble, non-fibrous inorganic filler, characterized by the fact that it contains from 1% to 30% of fibers, from 60% to 95% of filler and from 2% to 30% of organic polymer.

10. The water-laid sheet of Claim 9 characterized by the fact that the organic polymer is derived from ethylenically unsaturated monomers by emulsion polymerization and has in latex form a bound charge of from 0.03 to 0.4 milliequivalent per gram of polymer.

## Patentansprüche

1. Verfahren zur Herstellung einer hoch gefüllten Faserfolie mit den folgenden Stufen:
(I) Herstellung einer wäßrigen Dispersion von wasserdispergierbaren Fasern;
(11) Mischen dieser Dispersion mit:
(A) einem fein verteilten, im wesentlichen wasserunlösichlen, nicht faserförmigen anorganischen Füller; und
(B) einem Bindemittei, das ein filmbildendes, wasserunlösliches organisches Polymeres in Form eines ionisch stabilisierten Latex enthält;
(III) kolloidale Destabilisierung der entstehenden Mischung zur Bildung eines Faseragglomerats in wäßriger Suspension;
(IV) Verteilung und Entwässerung der wäßrigen Suspension auf einem porösen Träger zur Bildung eines feuchten Gewebes; und
(V) Trocknung des Gewebes;
dadurch gekennzeichnet, daß die nach Stufe (II) erhaltene Mischung enthält:
1 bis 30% Fasern,
60 bis 95% Füllstoff,
2 bis 30% Latex,
wobei die Prozentangaben auf dem Trockengewicht basieren und auf das Gesamttrockengewicht bezogen sind, und dem ionisch stabilisierten Latex eine zur Beeinträchtigung der Bildung eines Faseragglomerates ausreichende, nicht ionische Stabilisierung fehlt.

2. Verfahren nach Anspruch 1, dadurch gekennzeichnet, daß die kolloidale Destabiliserungsstufe ein Faseragglomerat in wäßriger Suspension bildet, mit der Eigenschaft, daß die Suspension bei einer Konzentration von 100 g Feststoffe in 13 500 ml während einer Zeitspanne von ca. 4 Sekunden bis ca. 120 Sekunden in einer 10 inch (25,4 cm)x12 inch (30,5 cm)-Williams-Standard-Folien-Form (Sheet Mould) mit einem 2 inch (5,1 cm)-Ausiaß und einem 30 inch (76,2 cm)-Wasserleitungszweig, die mit einem 100 mesh (0,149 mm)-rostfreiem Stahl-Sieb mit einem Drahtdurchmesser von 0,0045 inch (0,0114 cm) versehen ist, so entwässert, daß beim Entwässern nach Stufe (IV) im feuchten Gewebe mindestens 85% der gesamten Feststoffe des Faseragglomerates, die mindestens 60% der Füllstoffe enthalten, zurückbleiben..

3. Verfahren nach Anspruch 1, dadurch gekennzeichnet, daß das organische Polymere im Latex eine gebundene Ladung von weniger als 0,7 Milliäquivalent pro Gramm Polymer besitzt.

4. Verfahren nach Anspruch 3, dadurch gekennzeichnet, daß das organische Polymere im Latex eine gebundene Ladung von 0.3 bis 0,4 Milliäquivalent pro Gramm Polymer besitzt.

5. Verfahren nach Anspruch 2, dadurch gekennzeichnet, daß die wäßrige Dispersion der Fasern eine Konsistenz von 0,1 bis 6% besitzt, die Fasern Zellulosefasern sind und das Faseragglomerat eine Entwässerungszeit von 15 bis 60 Sekunden besitzt.

6. Verfahren nach Anspruch 1, dadurch gekennzeichnet, daß die Menge der Fasern 5 bis 15% beträgt, die Menge des Füllstoffs 70 bis 90%, und der Latex copolymerisiertes Styrol und Butadien enthäit.

7. Verfahren nach Anspruch 1, dadurch gekennzeichnet, daß der Latex eine Mischung von mindestens zwei verschiedenen Latexzusammensetzungen ist und mindestens einer der Latices ein Copolymer aus einer äthylenisch ungesättigten Carbonsäure enthält.

8. Verfahren nach Anspruch 1, dadurch gekennzeichnet, daß die Destabilisierungsstufe durchgeführt wird durch Mischen des Produktes der Stufen (I) und (II) mit einer ausreichenden Menge einer wasserlöslichen oder wasserdispergierbaren, ionischen Verbindung oder eines Polymers, die eine in bezug auf die ionische Stabilisierung des Latex entgegengesetzte Ladung besitzen.

9. Wassergegossene, selbsttragende Folie, die im wesenlichen aus einer Mischung aus (A) wasserdispergierbaren Fasern, (.B) einem filmbildenden, wasserunlöslichen organischen Polymeren und (C) wasserunlöslichen, nicht faserförmigen anorganischen Füllstoffen- besteht, dadurch gekennzeichnet, daß sie 1 bis 30% Fasern, 60 bis 95% Füllstoff und 2 bis 30% organisches Polymeres enthält.

10. Wassergegossene Folie nach Anspruch 9, dadurch gekennzeichnet, daß das organische Polymere durch Emulsionspolymerisation eines äthylenisch ungesättigten Monomeren erhalten ist und in seiner Latexform eine gebundene Ladung von 0,03 bis 0,4 Milliäquivalent pro Gramm Polymeres besitzt.

## Revendications

1. Procédé de préparation d'une feuille fibreuse fortement chargée comprenant les stades suivants:
(1) obtention d'une dispersion aqueuse de fibres dispersables dans l'eau;
(II) mélange de ladite dispersion avec:
(A) une charge minérale, non fibreuse, finement divisée, presque insoluble dans l'eau; et
(B) un liant contenant un polymère organique filmogène, insoluble dans l'eau, sous la forme d'un latex stabilisé par des ions;
(III) déstabilisation du mélange résultant par des colloides pour former un agglomérat fibreux en suspension aqueuse;
(IV) répartition et égouttage de ladite suspension aqueuse sur un support. poreux pour former une feuille continue humide; et
(V) séchage de la feuille continue;
caractérisé par le fait que le mélange obtenu dans le stade (II) contient:
de 1 à 30% de fibres
de 60 à 95% de charge
de 2 à 30% de latex
lesdits pourcentages étant basés sur le poids de la matière sèche, calculés sur le poids total des matières sèches, et que le latex stabilisê par des ions est dépourvu de stabilisation suffisamment non- ionique pour interférer avec la formation d'un agglomérat fibreux.

2. Procédé selon la revendication 1, caractérisé par le fait que le stade de déstabilisation par des colloi des forme un agglomérat fibreux en suspension aqueuse avec les propriétés suivantes: pour une concentration en matières solides de 100 g dans 13 500 millilitres, la suspension s'égouttera en un temps d'environ 4 secondes à environ 120 secondes dans un moule pour feuille, normalisé, "William" (Williams Standard Sheet Mould) de 25,4 cm (10 inches) par 30,5 cm (12 inches), comportant une sortie de 5,1 cm (2 inches) et une colonne d'eau de 76,2 cm (30 inches). et muni d'un tamis en acier inoxydable ayant un vide de maille de 0,149 mm (100-mesch) et un diamètre du fil de 0,0114 cm (0,0045 inch) de sorte que, lors de l'égouttage au stade (IV), on retient dans la feuille continue humide au moins 85% des matières solides totales provenant de l'agglomérat fibreux comprenant au moins 60% en poids de la charge.

3. Procédé selon la revendication 1, caractérisé par le fait que le polymère organique dans le latex a moins de 0,7 milliéquivalent de charge liée par gramme de polymère.

4. Procédé selon la revendication 3, caractérisé par le fait que le polymère organique dans le latex a une charge liée de 0,3 à 0,4 milliéquivalent par gramme de polymère.

5. Procédé selon la revendication 2, caractérisé par le fait que la dispersion aqueuse des fibres a une consistance de 0, 1 % à 6%, que les fibres sont des fibres cellulosiques et que l'agglomerat fibreux a un temps d'égouttage de 15 à 60 secondes.

6. Procédé selon la revendication 1, caractérisé par le fait que la quantité de fibres est de 5 à 15%, la quantité de charge est de 70% à 90% et que le latex contient du styrène et du butadiène copolymérisés.

7. Procédé selon la revendication 1, caractérisé par le fait que le latex est un mélange d'au moins deux compositions différentes de latex et qu'au moins un des latex contient un copolymère d'un acide carboxylique éthyléniquement insaturé.

8. Procédé selon la revendication 1, dans lequel le stade de déstabilisation est effectué en mélangeant avec le produit des stades (1) et (II) une quantité suffisante d'un composé ou d'un polymère, ioniques, solubles dans l'eau ou dispersables dans l'eau, ayant une charge de signe opposé à celui de la stabilisation ionique du latex.

9. Feuille auto-supportée, déposée par l'eau, constituée essentiellement par un mélange de (A) fibres dispersables dans l'eau, (B) un polymère organique, filmogène, insoluble dans l'eau, et (C) une charge minérale non-fibreuse, insoluble dans l'eau, caractérisée par le fait qu'elle contient de 1 % à 30% de fibres, de 60% à 95% de charge et de 2% à 30% de polymère organique.

10. Feuille déposée par l'eau selon la revendication 9, caractérisé par le fait que le polymère organique provient de monomères éthyléniquement insaturés par polymérisation en émulsion et comporte sous forme de latex une charge liée de 0,03 à 0,4 millléo tivalent par gramme de polymère.
